

W. M. FULTON,  
PROCESS OF TEMPERING CORRUGATED WALLS,  
APPLICATION FILED NOV. 20, 1916.

1,293,078.

Patented Feb. 4, 1919.



Fig. 1.



Fig. 2.



Fig. 3.



Fig. 4. *By* Maurice Cameron, Lewis & Massie  
Attorneys

Inventor

Weston M. Fulton.

# UNITED STATES PATENT OFFICE.

WESTON M. FULTON, OF KNOXVILLE, TENNESSEE, ASSIGNOR TO THE FULTON COMPANY, OF KNOXVILLE, TENNESSEE, A CORPORATION OF MAINE.

## PROCESS OF TEMPERING CORRUGATED WALLS.

1,293,078.

Specification of Letters Patent.

Patented Feb. 4, 1919.

Application filed November 20, 1916. Serial No. 132,461.

*To all whom it may concern:*

Be it known that I, WESTON M. FULTON, a citizen of the United States of America, and a resident of Knoxville, Tennessee, have 5 invented a new and useful Improvement in Processes of Tempering Corrugated Walls, which invention is fully set forth in the following specification.

This invention relates to a process of 10 hardening and tempering a corrugated wall, and is particularly adapted to the production of such walls for use in collapsible and expandible vessels designed to confine fluids under pressure.

15 It has for an object the production of corrugated walls of high resilience, of great strength and durability, and which can be collapsed and expanded many times substantially without injury thereto.

20 Flexible corrugated walls of the type referred to are repeatedly subjected to tensional, compression and bending stresses. If they be constructed of soft steel, these stresses soon produce crystallization and 25 fracture at the curved portions of the corrugations, owing to frequent straining of the metal beyond its elastic limit. It is an object of this invention to so harden and temper the portions of the corrugations subjected to the greater stresses as to render 30 these walls more durable and resistant to strains while securing a proper degree of resiliency therein.

A further object of this invention is to 35 provide a hardening and tempering process wherein different portions of the wall have different degrees of hardness. Other objects will appear as the description of the invention proceeds.

40 Stated briefly, the invention comprises the process of hardening and tempering a corrugated wall which consists in heating said wall and subjecting the same to a cooling medium while said wall is differentially 45 protected from said medium, whereby different portions of said wall are brought to their final cooled condition at different rates, resulting in different degrees of hardness.

The inventive idea involved is capable of 50 a variety of expressions, one of which, for the purpose of illustration, is hereinafter specifically described, but it is to be expressly understood that such illustration is not intended as a definition of the limits of the in-

vention, reference being had to the appended 55 claims for that purpose.

On the accompanying drawings, appropriate apparatus is illustrated for the carrying out of the process, but it is to be understood that such apparatus has been selected 60 for the purpose of illustration only and is in no respect definitive of the scope of the invention, as the invention idea is not dependent on any particular apparatus for the performance of the process, any suitable apparatus being within the purview of the invention.

Referring in detail to the drawings, wherein the same reference characters designate corresponding parts in the several 70 figures—

Figure 1 is a vertical cross section of a corrugated wall provided with heat-absorptive means in accordance with the present invention;

Fig. 2 is a plan of one of the top and bottom clamping members;

Fig. 3 is a plan of a ring designed to be positioned within a space between adjacent corrugations opening exteriorly of the wall; 80 and

Fig. 4 is a plan of a ring designed to be positioned within a space between adjacent corrugations opening interiorly of the wall.

In accordance with the present invention, 85 a metal blank, preferably of a good grade of steel, is corrugated in any suitable way while in its softest state, the same being annealed frequently to withdraw temper unavoidably formed therein by the working 90 of the metal.

The corrugated wall is then provided with heat-absorptive means in contact with those portions of the wall which are subject to less strain than other portions thereof, such 95 heat-absorptive means being maintained out of contact with those portions which it is desired shall be harder or more highly tempered. In the form shown (Fig. 1), metal blocks 1 and 2, in the form of rings, are 100 positioned between and in contact with the lateral or flat portions of a corrugated wall 3, said rings not contacting with the portions of said corrugations constituting the bends therein. Said rings are preferably 105 of a thickness equal to the distance between adjacent lateral walls of the corrugations when said wall is in its unstressed condition,

The rings fitting into the spaces between lateral portions of the corrugations which open exteriorly of the wall may desirably be made in two sections 4 and 5, as shown (Fig. 3). The rings fitting into the spaces between lateral portions of the corrugations which open interiorly of the wall may desirably be made in six sections 6, 7, 8, 9, 10 and 11, as illustrated (Fig. 4). The wall 3, 10 with interposed rings 1 and 2, is then clamped firmly between end clamping-rings 12 and 13 in any suitable manner, as by a through-bolt 14 passing through central apertures 15 in the upper and lower clamping-rings and receiving on its threaded end 16 a nut 17. As shown, said clamping-rings are provided with a plurality of apertures 18, whereby the cooling medium may have free access to the interior of the wall. 15

20 The corrugated wall, with its interposed rings of heat-absorptive material, is then heated until the same is brought to an appropriate temperature, preferably that corresponding to a dull-red heat. The wall and 25 heat-absorptive means in contact therewith are then immersed in a chilling bath, preferably of oil. The portions of the wall out of contact with the heat-absorptive rings are quickly chilled by the bath and thereby 30 given a high degree of hardness or temper. The lateral walls of the corrugations which are in contact with the heat-absorptive rings are protected from the chilling effect of the bath and, owing to the gradual giving up of 35 heat by the rings, such portions of the wall are hardened to a less extent or may be left substantially without temper. Furthermore, the delivery of heat by the interposed rings to the portions of the corrugations in contact therewith affects the adjacent portions 40 of the corrugations which are out of contact with the heat-absorptive means, thereby drawing the temper therein but to different degrees in accordance with the distance from 45 the portions in contact with the aforesaid rings. Thereby is there no abrupt change of temper or hardness between the lateral walls and the curved walls of the corrugations.

By the use of heat-absorptive rings of a 50 thickness equal to the space between adjacent lateral walls, and by the clamping of the corrugated wall between such heat-absorptive rings, the vessel is firmly supported during the hardening or tempering process 55 with a consequent prevention of the wall becoming distorted or warped in any way during the subsequent chilling of the same.

60 While the process has been described as applied only to hardening and tempering of the bends of the corrugations, it will be apparent that, by the selection of appropriate material and rings of appropriate size and shape, more or less of the corrugated walls may be hardened and tempered and the range 65 and gradation of temper may be suitably

varied in accordance with the nature of the material used in the wall and with the uses to which such wall is to be put. The invention, therefore, is not to be restricted to hardening and tempering the bends only of the 70 corrugations nor to the use of heat-absorptive means of the shape, size or kind illustrated on the drawings, the invention being directed broadly to differentially protecting the corrugated wall from the medium of 75 the chilling bath by any suitable means to the end that the unprotected portions of the wall shall be materially hardened, the protected portions rendered less hard, and the gradation of hardness or temper formed at 80 the junction between the harder and less hard portions of the wall, said protection being preferably afforded by heated heat-absorptive means which by differential delivery of heat to the wall draws more or less 85 of the temper from the hardened portions and insures the aforesaid gradation of hardness.

What is claimed is:

1. The process of differentially hardening 90 and tempering a corrugated wall which comprises maintaining heat-absorptive means in contact with the lateral walls of the corrugations but out of contact with the bends thereof, heating said corrugated wall and 95 heat-absorptive means, and subjecting the whole to a cooling medium.

2. The process of differentially hardening and tempering a corrugated wall which comprises interposing metal blocks between 100 and in contact with the lateral walls of the corrugations but out of contact with the bends thereof, heating said corrugated wall and blocks, and subjecting the whole to a cooling medium.

3. The process of differentially hardening and tempering a corrugated wall which comprises maintaining heat-absorptive means in contact with portions of the walls of the corrugations but out of contact with 110 other portions thereof, heating said corrugated wall and heat-absorptive means, and subjecting the same to a cooling medium.

4. The process of differentially hardening and tempering a corrugated wall which 115 comprises heating said wall, and subjecting the same to a cooling medium while retarding the cooling of portions of said wall and producing a gradation of hardness in other portions of said wall.

5. The process of differentially hardening and tempering a corrugated wall which comprises heating said wall with heat-absorptive means in contact with the lateral portions thereof, and subjecting the whole to 125 a cooling medium.

6. The process of differentially hardening and tempering a corrugated wall which comprises heating said wall, and subjecting the same to a cooling medium with means 130

in contact with the lateral portions of said wall to prevent the rapid chilling of such portions.

7. The process of differentially hardening and tempering a corrugated wall which comprises heating said wall, and subjecting the same to a cooling medium with heated means in contact with portions of said wall to draw the temper in other portions of said

10 wall.

8. The process of differentially hardening and tempering a corrugated wall which comprises heating said wall, and subjecting the same to a cooling medium with heated 15 means in contact with portions of said wall to control the cooling of the same and to give up heat to other portions of said wall.

9. The process of making a corrugated steel wall which comprises corrugating a 20 blank of soft steel, and differentially hardening and tempering the same by heating said wall and subjecting the same to a cooling medium while retarding the cooling of portions of said wall and producing a gradation 25 of hardness in other portions of said wall.

10. The process of making a corrugated steel wall which comprises corrugating a blank of soft steel, and differentially hardening and tempering the same by heating 30 said wall with heat-absorptive means in contact with the lateral portions thereof and subjecting the whole to a cooling medium.

35 11. The process of making a corrugated steel wall which comprises corrugating a blank of soft steel, maintaining heat-absorptive means in contact with portions of the walls of the corrugations but out of contact with other portions thereof, heating said

40 corrugated wall and heat-absorptive means and subjecting the same to a cooling medium.

12. The process of making a corrugated

steel wall which comprises corrugating a 45 blank of soft steel, maintaining heat-absorptive means in contact with the lateral walls of the corrugations but out of contact with the bends thereof, heating said corrugated wall and heat-absorptive means, and subjecting 50 the whole to a cooling medium.

13. The process of making a corrugated steel wall which comprises corrugating a blank of soft steel, interposing metal blocks between and in contact with the lateral walls 55 of the corrugations but out of contact with the bends thereof, heating said corrugated wall and blocks, and subjecting the whole to a cooling medium.

14. The process of making a corrugated steel wall which comprises corrugating a blank of soft steel, and differentially hardening and tempering the same by heating said wall and subjecting the same to a cooling medium with means in contact with the lateral portions of said wall to prevent the rapid chilling of such portions.

15. The process of making a corrugated steel wall which comprises corrugating a blank of soft steel, and differentially hardening and tempering the same by heating said wall and subjecting the same to a cooling medium with heated means in contact with portions of said wall to draw the 70 temper in other portions of said wall.

16. The process of making a corrugated steel wall which comprises corrugating a blank of soft steel, and differentially hardening and tempering the same by heating said wall and subjecting the same to a cooling medium with heated means in contact with portions of said wall to control the 80 cooling of the same and to give up heat to other portions of said wall.

In testimony whereof I have signed this 85 specification.

WESTON M. FULTON.